

# UNITED STATES PATENT OFFICE.

ROY G. TELLIER, OF CHICAGO, ILLINOIS.

## EARTH-TREATING PROCESS AND PRODUCT.

1,402,112.

Specification of Letters Patent.

Patented Jan. 3, 1922.

No Drawing.

Application filed November 12, 1920. Serial No. 423,710.

To all whom it may concern:

Be it known that I, Roy G. TELLIER, a citizen of the United States, residing in the city of Chicago, in the county of Cook and State of Illinois, have invented new and useful Improvements in Earth-Treating Processes and Products, of which the following is a specification.

My invention relates to the treatment of materials, such as fuller's earth, or other earths of similar characteristics, used for filtering, de-colorizing, purifying and otherwise acting upon fluids or liquid substances, such as oils in general, and particularly vegetable and animal fats and oils, and mineral or petroleum oils, in order to dissolve or oxidize impurities therein, and prevent objectionable colloidal conditions arising in the clay when brought into contact with the oils in the de-colorizing and purifying processes.

A general object of my invention is to so treat the earth, such as those referred to, and particularly fuller's earth, to increase the oil bleaching and purifying properties thereof, and that it shall by virtue of the treatment, avoid or overcome colloidal and oil absorption tendencies when coming into contact with the oils to be acted upon, and therefore will filter faster and retain less oil than heretofore when used in bleaching, de-colorizing, filtering, purifying and otherwise acting upon fluids and liquids, such as oils in general; and to increase the durability of the earth for repeated use in de-colorizing, purifying and filtering mineral oils so that it shall be put into condition that it shall better withstand or otherwise improve it for further treatment after having been used upon mineral oils and liquid substances.

My invention also resides in the improved material herein described and in the process of producing the same.

I shall take the treatment of fuller's earth found in Bexar and Medina Counties, State of Texas, known as Medina fuller's earth, for illustrative purposes and as the preferred form of my invention. This fuller's earth, for example, as it has heretofore been treated, is first dried in a neutral atmosphere ranging from 250 to 400 degrees Fahrenheit so that it may be readily ground, or divided, (which temperatures only serve to drive off the free moisture,) and then screened to a range of sizes as will pass a 200 mesh screen for vegetable and animal fats and oils; and

through a 15 mesh screen, but will not pass through an 80 mesh screen, for mineral and petroleum oils. After this treatment, as heretofore carried out and above described, the earth is ready for use upon oils.

It is well known that, ordinarily, fuller's earth when so finely ground or divided that it will pass through a 200 mesh screen presents the most extensive surfaces to the oils to be acted upon and therefore possesses the maximum of bleaching properties; but as is also well known, all clays, or fuller's earths, when so finely ground for use in bleaching and filtering oils retains and absorbs more oil than clays not so finely ground, and it is therefore desirable to avoid using clays in this finely divided condition if possible to obtain the proper or standard bleach without so doing. However, it is even more objectionable to use the clays, or fuller's earths,

in the preferred form of my invention, when so finely ground and treated as above outlined, because of its peculiar physical structure which causes it to disintegrate and to become colloidal, structureless, sluggish and flocculent and indisposed to diffuse or suspend itself in the oils in the bleaching and purifying process under the form of treatment above outlined and as heretofore practiced, which makes it not only difficult to bring the clays into contact with the oil, but tends to form in a slightly gelatinous or flocculent mass in the agitating vats, filters and filter-presses, and therefore presents filtration troubles and also absorbs and retains the maximum of oil when used in the de-colorizing and purifying processes during filtration. Under such old methods of treatment the clays would also re-absorb detrimental moisture in storage before use which greatly detracts from its bleaching properties and therefore greatly lessens the value of such earths for use in treating animal and vegetable oils and fats as above enumerated.

Now I have discovered that it is possible to economically increase the bleaching, de-colorizing and purifying properties of fuller's earths, and to prevent this tendency towards colloidalility therein by changing the physical structure or conditions of the clay without destroying its chemical efficiency and thereby hasten filtration and greatly reduce the objectionable oil retention tendencies and to prevent the clay from re-absorbing

an excess of detrimental moisture in storage without in anywise injuriously affecting the character of the material under treatment, by subjecting the same to a heating or low 5 baking temperature in a current of air which thoroughly dissolves or oxidizes and neutralizes the impurities out of the clay which tend to retard and interfere with the natural bleaching functions of the earth, 10 and at the same time removes nearly, but not quite, all of the combined water and produces other changes which creates it into a material of granular structure with the maximum of porosity, and not only increases its durability for repeated use for 15 mineral and petroleum oil uses, but greatly lessens its tendency to absorb moisture while in storage before actually using the same.

In the practice of my process in its preferred form, considering for the purpose of illustration, its application to fuller's earth or clay, the earth on being received at the place of treatment is first reduced, or crushed into small lumps, the largest of which not 25 to exceed one half inch in diameter. When so crushed the material is artificially and thoroughly dried in any of the well known methods so that all the free moisture shall be removed so that the earth may be readily 30 ground, or divided, into any size mesh desired. For vegetable and animal fats and oils it is desirable for reasons already stated, to avoid the necessity of having to use a material that will all pass through a 200 35 mesh screen, and by my improved method of treatment a material ground, or divided, so that it will all pass through a 100 mesh screen, but not all through a 150 mesh screen, will yield an improvement of 25% 40 in bleaching qualities, and at the same time filter faster and absorb at least 20% less oils than the same earthy materials would under the treatment heretofore practiced.

After grinding or dividing the earth into 45 the mesh desired it is now ready for its final oxidizing and partially dehydrating treatment. The furnace or heater used for this treatment should preferably be of the rotary, inner-flue, highly oxidizing type to 50 prevent the carbon dioxide resulting from the combustion of fuel to come into direct contact with the material, which affects the earth injuriously. I find that the best results are obtained by causing the earth particles to be set in motion relative to each other and in suspension, or partial suspension, and heating the earths in an artificially supplied current, or currents, of air until they are thoroughly oxidized and 55 nearly, but not quite, all of the combined water is driven off. Complete oxidization is indicated by a complete change in the color of the earth, either to a pale yellow or slightly golden, or a mouse colored gray. 60 65 The color depending somewhat on the ex-

tent to which the oxidizing and dehydrating process may have been carried out in the pre-drying of the clays in the coarse lumps as they come from the crusher. To bring about complete oxidization there must be a constant supply of fresh air waves continually scattered to all parts of the heating chamber while the mass of grains are kept in constant motion and suspension, or partial suspension in the heating chamber during treatment to enable the heat and air to uniformly come in contact with all the grains. An adequate amount of air can be cheaply and easily supplied to any of the well known rotary type of drier by a power 70 driven blower, compressed air or natural draft, preferably pre-heated so as to insure even distribution or dissemination of the air currents to all parts of the chamber. As air supplied in the manner indicated is 75 cheaply accomplished an excess would, of course, be better than a deficiency up to the point where it would begin to blow the material out of the heating chamber.

The temperature of this oxidizing or heating chamber should range, for vegetable and animal fats and oil uses, from 700 to 900 degrees Fahrenheit, and from 850 to 1350 degrees Fahrenheit for mineral oil use. The time required for treatment and complete 80 oxidization and sufficient de-hydration varies, of course, in accordance with the size of grains treated. I find that for vegetable and animal fats and oil uses the time varies from 10 to 25 minutes, and for mineral and 85 petroleum oil uses from 15 to 35 minutes. This variance depending entirely on the temperature employed and on the extent to which the mass of grains are kept in motion or suspension and thus uniformly exposed 90 to the heat and air.

It may here be noted that while I have described in considerable detail a specific manner of carrying out my new process of treating fuller's earth, or clays, it is to be understood that this description is illustrative only and for the purpose of making clear the principles underlying the invention. Quite similar results can be obtained by carrying out the oxidizing and dehydrating 100 treatment in the heat and air currents in the initial drying of the clays as they come from the crusher in their lump form of one half inch or less in diameter. To secure the improvement in this manner, however, the temperature and time employed and the velocity of air currents supplied must greatly exceed that employed in the methods heretofore outlined. Of necessity the bulk of the weight of these lumps would be on the interior of these lumps and would consequently not be readily subjected to the oxidizing influences of the heat and air currents without the use of temperatures ranging from 900 to 1350 degrees Fahrenheit or 110 115 120 125 130

more, and as much air current as it is possible to apply without blowing the particles of clay out of the heating chamber, and correspondingly increasing the length of time of treatment.

My improved method of treating fuller's earth, or earthy material, completely changes the physical structure of the earth and produces a flaky and active condition in the material which, when brought into contact with the oils to be treated, readily goes into suspension and freely diffuses itself throughout the mass of the oil which permits each particle of clay to do its maximum of work and at the same time permits of the freest filtration and the minimum of oil absorption, and produces the maximum of bleach in the de-colorizing and purifying processes.

What I claim, is:

1. A process for forming a filtering and oil de-colorizing and purifying material, which consists in completely oxidizing and partially baking a fuller's earth, while the particles thereof are in motion relative to each other, at a temperature between 700 and 1350 degrees Fahrenheit in a current of air.

2. A process for forming a filtering and oil de-colorizing and purifying material which consists in removing all the free moisture, or water, in fuller's earth; granulating the same to desired size by mechanical means; then oxidizing and partially baking such earthy material in suspension in a current of air at a temperature to drive off a part of the combined water and storing the same.

3. A process for forming a filtering and oil de-colorizing and purifying material which consists in removing all the free moisture, or water in fuller's earth; granulating the same to desired size by mechanical means; then oxidizing and baking such earthy material in suspension in a current of air at a temperature to drive off a part of the combined water and storing the same.

4. A process for forming a filtering and oil de-colorizing and purifying material which consists in removing all the free water in fuller's earth; granulating the same to desired size by mechanical means; then oxidizing and baking such earthy material in a current of air while the particles thereof are in motion relative to each other at a temperature to drive off a part of the combined water and storing the same.

5. A process of treating, maintaining or improving the efficiency of fuller's earth, or earthy material of similar characteristics, for use in filtering, de-colorizing and purifying oils, which consists in heat treating or partially baking the fuller's earth in a current of air while the particles thereof are in motion relative to each other at a temperature which drives off a part of the chemically combined water, which oxidizes and

neutralizes ingredients of said earth, or earthy material, tending to retard and hinder its bleaching properties.

6. The process of treating, maintaining or improving the efficiency of fuller's earth, or earthy material of similar characteristics, for use in filtering, de-colorizing and purifying oils, which tends toward colloidal and oil absorption in the de-colorizing and purifying process, which consists in heat treating or partially baking the fuller's earth in a current of air while the particles thereof are in motion relative to each other which completely oxidizes or neutralizes ingredients of said earth or earthy material tending to retard or hinder its bleaching properties, and which changes the physical structure of said earth, or earthy material.

7. The process of treating, maintaining or improving the efficiency of fuller's earth, or earthy material of similar characteristics, for use in filtering, de-colorizing and purifying oily liquid, which tends toward colloidal and oil absorption in the de-colorizing and purifying process, which consists in heat treating, or baking, the fuller's earth in a current of air while the particles thereof are in motion relative to each other at a temperature ranging from 700 degrees Fahrenheit to 1350 degrees Fahrenheit which changes the physical structure of the clays and increases the degree of dispersion and diffusion of the clay throughout the mass of oil in the de-colorizing and purifying process which reduces oil absorption tendencies and hastens filtration.

8. A process for treating fuller's earth, or like material, for use in filtering, de-colorizing and purifying oils and oily liquid which consists in granulating such earth; heating or partially baking such earth while the granules thereof are in motion relative to each other and partially suspended so as to permit free circulation of air currents, supplied in any well known manner, between the particles of the earth while the same are in motion and partial suspension; the heating or baking being conducted at a temperature of from 700 to 1350 degrees Fahrenheit.

9. The herein described process which consists in treating fuller's earth, or earthy material of similar characteristics, for use in filtering, de-colorizing and purifying oily liquid, by first drying said earth to remove all free moisture, then reducing said earth to suitable size by mechanical means, then heat treating and partially baking said fuller's earth while the particles thereof are in motion relative to each other, in a current of pre-heated air until completely oxidized and nearly all the chemically combined water is driven off.

10. A process for treating fuller's earth, or like material, for use in filtering, de-colorizing and purifying oils and oily liquid,

- which consists in granulating such earth to desired size, conveying the earth to an apparatus permitting the granules thereof to be set in motion relative to each other and partially suspended in a preheated, oxidizing atmosphere until the earth becomes substantially oxidized and a part of the chemically combined water is driven off.
11. A process of treating fuller's earth, or other earthy material of similar characteristics, for use in filtering, de-colorizing and purifying oily liquid, by first drying said earth to remove all free moisture; then reducing said earth to suitable size by mechanical means; then conveying the same to an apparatus permitting such earth to be freely gravitationally dropped down through a pre-heated, oxidizing atmosphere at a temperature between 700 and 1350 degrees Fahrenheit; discharging free individual currents of air against the falling material during its gravitational passage through the apparatus, so that the material will become completely oxidized and nearly, but not quite all, the chemically combined water is driven off.
12. A process of treating fuller's earth, or other earthy material of similar characteristics, for filtering, de-colorizing and purifying oily liquids, by first drying said earth to remove all free moisture; then reducing said earth to suitable size by mechanical means; conveying said granulated earth un-
- der treatment to an apparatus permitting such granules to be set in motion relative to each other in the oxidizing action of heat and air currents, continually heating such earth until oxidized and a part of the chemically combined water is driven off.
13. A method of preparing fuller's earth, or like material, for use in filtering, de-colorizing and purifying oil and oily liquid, which consists in setting such earth in motion, agitation and suspension; projecting currents of air therein, in any well known manner; continually heating or baking the earth at a temperature until it is oxidized and part of the combined water is driven off, grinding or granulating to desired size for use.
14. A method of preparing fuller's earth, or like material, for use in filtering, de-colorizing and purifying oil or oily liquid, which consists in conveying such earth to an apparatus permitting such earth to be set in motion, agitation and suspension; projecting currents of air therein in any well known manner; continually heating or baking the earth at a temperature until it is oxidized and all the free or uncombined water is driven off, but not all the chemically combined water; granulating or grinding to desired size for use.

ROY G. TELLIER.

In the presence of—

N. CONOVER,  
W. J. McLAUGHLIN.